

1

3,177,144

## LUBRICATING COMPOSITION

Thomas E. Reamer, El Cerrito, and John E. Weigel, Berkeley, Calif., assignors to Shell Oil Company, New York, N.Y., a corporation of Delaware  
No Drawing. Filed Jan. 23, 1961, Ser. No. 83,947

6 Claims. (Cl. 252—32.5)

This invention relates to aqueous base, metal-working lubricating compositions. More particularly, it relates to extreme pressure water-base metal cutting fluids for use in cutting, drilling, reaming, grinding and other machining and forming operations of ferrous and non-ferrous metals.

It is known that water-base cutting fluids possess good cooling properties, but that they lack the lubricating and extreme pressure properties of oil base lubricants. On the other hand, oil base lubricants are inferior coolants and cause odor, smoke, and staining.

The art discloses various water-base cutting fluids, most of which lack extreme pressure properties. Because of the multiplicity of additives which the majority of such fluids contain, they are unstable, tend towards phase separation and foaming, and are difficult and expensive to prepare. Among the materials commonly used in such water solutions are an alkali, e.g., borax, sodium carbonate or trisodium phosphate, an anti-rust agent, e.g., sodium nitrite or triethanolamine, and wetting, buffering and solubilizing agents. The metal wetting additives may be water-soluble non-ionic compounds such as a reaction product of alkylphenol-ethylene oxide or a block polymer of ethylene oxide and propylene oxide sold commercially under the trade name of "Pluronics" (Wyandotte Chemical Company).

It is an object of this invention to provide a metal-working aqueous base lubricant having both good cooling and good lubricating properties. Another object of the invention is to provide a non-corrosive water-base cutting fluid. Still another object of the invention is to provide a stable water-base cutting fluid useful at high speeds, elevated temperatures, heavy loads and extreme pressures.

The above and other objects are attained by the present invention which provides a metal-working lubricant of an aqueous base such as water to which is added a small amount (0.5-15%) of a new and novel compound, namely, a water-soluble (di)alkali metal salt of chloro  $C_{1-4}$  alkyl phosphonic acid. Water base solutions of this type form excellent extreme pressure metal working lubricants. Such solutions are particularly compatible with certain additives to produce a still more effective metal working lubricant. Such a formulation may comprise an aqueous base such as water to which is added from about 0.5% to about 15%, preferably from about 2% to about 10% by weight each of (1) a water-soluble (di)alkali metal salt of chloro  $C_{1-4}$  alkyl phosphonic acid, (2) an alkanolamine salt of a  $C_{12-20}$  saturated or unsaturated fatty acid, (3) a free alkanolamine and (4) a water-soluble heterocopolymeric alkylene glycol, ether or ester thereof, wherein the different oxyalkylene units are substantially randomly distributed throughout the entire polyoxyalkylene chain. The final water base fluid should have a pH between 8 and 11, preferably from about 9 to about 10. This is accomplished by addition of excess base (alkali hydroxide, e.g., NaOH) used in forming the phosphonate salts.

The combination of the above essential additives functions in a particular manner and produces an outstanding metal working fluid. The normal alkali metal chloro  $C_{1-4}$  alkyl phosphonate functions as an extreme pressure and load carrying agent. The alkanolamine carboxylate decreases bearing wear and grease loss. The free alkanolamine inhibits metal corrosion, particularly of ferrous metals, without producing any undesirable side effects,

2

which is not the case with alkali metal nitrites, chromates, borates, etc., which are toxic and under some conditions may promote corrosion. The water-soluble heteropolymer improves the antifrictional properties of compositions of the present invention, particularly under slow sliding conditions. On the other hand, other non-ionic polymeric compounds such as alkyl phenol-ethylene oxide reaction products, block copolymers of dissimilar alkylene oxides and their derivatives, produce undesirable frictional problems, foaming, instability and the like.

The (di)alkali metal chloro  $C_{1-4}$  alkyl phosphonate include sodium, potassium and/or lithium salts of said acid, which acid portion of the salt can be represented by the general formula

15



where R is a  $C_{1-4}$  alkyl radical, preferably a  $C_{1-2}$  alkyl radical such as methyl or ethyl radical and the chlorine atom (Cl) is in the alpha position relative to the phosphorous atom and A is an alkali metal anion as defined. Examples of such compounds include disodium chloromethyl phosphonate, disodium alpha-chloroethyl phosphonate, disodium alpha-chlorobutyl phosphonate, dipotassium chloromethyl phosphonate, dipotassium alpha-chloroethyl phosphonate, dipotassium alpha-chlorobutyl phosphonate, dipotassium alpha-chloroisopropyl phosphonate, dilithium chloromethyl phosphonate, dilithium alpha-chloromethyl phosphonate, dilithium alpha-chloro-propyl phosphonate and mixtures thereof. A small excess of alkali hydroxide is used so that the pH of the water solution is above 8.

The alkanolamines include mono-, di- and triethanolamine, isopropanolamine, butanolamine, N,N-dimethyl-isopropanolamine and the like. These amines are also used to make the amine salts of  $C_{12-20}$  fatty acids such as lauric acid, palmitic acid, stearic acid, oleic acid, linoleic acid, linolenic acid, ricinoleic acid and the like. Preferred amine salts are triethanolamine oleate, triethanolamine ricinoleate and mixtures thereof.

The water-miscible heteropolymer polyalkylene oxide fluids enhance the cutting performance of the compositions of the present invention by enhancing metal wetting. The above oxides are heteropolymers of dissimilar alkylene oxides such as copolymer ethylene oxide and 1,2-propylene oxide [poly(oxyethylene-1,2-oxypropylene)glycol], as well as monoethers and monoesters thereof, preferably at oxide ratios of from 75:25 to 10:90 ethylene oxide to 1,2-propylene oxide, and molecular weight of from about 250 to about 1500.

By a ratio of from 75:25 to 10:90 is meant that, in the formation of copolymer the amount of 1,2-propylene oxide is from  $\frac{1}{3}$  to 9 times the amount of ethylene oxide present, by weight, the parts or proportions of the 1,2-propylene oxide being given last. These materials are described in U.S. Patents 2,425,755 and 2,425,845. The copolymer diols may be employed in a modified form as the monoethers or monoesters of monohydric alcohols or monobasic acids with the diols. Both the alcohols and the monocarboxylic acids preferably have from 1 to about 5 carbon atoms.

Minor amounts (0.01-1%) of anti-foaming, masking, bactericidal and anti-corrosive agents for ferrous metals, copper and copper alloys, and/or perfuming agents, may be added to improve the compositions of this invention. Among such materials may be included: anti-foaming agents, e.g., organic silicone compounds illustrated by dimethyl silicone polymer; phosphates, e.g., tributyl phosphate, alkali metal polyphosphates illustrated by sodium alkyl polyphosphates; masking agents, e.g., low molecular weight aldehydes (acetaldehyde); oil of pines, oil of

mirbane; bactericides, e.g., alkyl phenols and phenates such as sodium o-phenyl phenate; and copper anti-corrosion agents, e.g., mercaptobenzothiazoles (sodium mercaptobenzothiazole), and the like.

The following compositions are representative of the invention, which can be used neat or diluted with from 1 to 10 parts of water, as metal-working lubricants for cutting, drilling and the like. The proportions are given in percentages by weight.

| Composition A:                                                                                      | Percent | 10   |
|-----------------------------------------------------------------------------------------------------|---------|------|
| Dipotassium chloromethyl phosphonate                                                                |         |      |
|                                                                                                     |         |      |
| Oleic acid                                                                                          | 4.12    | 0.05 |
| Triethanolamine                                                                                     | 3.00    |      |
| Heterocopolymer of ethylene oxide-1,2-propylene oxide (72/25) having a viscosity of 1400 at 100° F. | 20      | 2.00 |
| Na o-phenylphenate                                                                                  |         | 0.05 |
| Na alkyl polyphosphate                                                                              |         | 0.02 |
| Na mercaptobenzothiazole                                                                            |         | 0.50 |
| Water                                                                                               | Balance | 25   |
| Composition B:                                                                                      |         |      |
| Dipotassium chloromethyl phosphonate                                                                | 5       |      |
| Triethanolamine oleate                                                                              |         | 0.1  |
| Triethanolamine                                                                                     |         | 1.5  |
| Heterocopolymer of ethylene oxide-1,2-propylene oxide (72/25) having a viscosity of 1400 at 100° F. | 30      | 3.0  |
| Water                                                                                               | Balance |      |
| Composition C:                                                                                      |         | 35   |
| Disodium chloromethyl phosphonate                                                                   | 4       |      |
| Triethanolamine oleate                                                                              |         | 0.1  |
| Triethanolamine                                                                                     |         | 1.5  |
| Heterocopolymer of ethylene oxide-1,2-propylene oxide (72/25) having a viscosity of 1400 at 100° F. | 40      | 3.0  |
| Water                                                                                               | Balance |      |
| Composition D:                                                                                      |         | 45   |
| Disodium chloromethyl phosphonate                                                                   | 4       |      |
| Triethanolamine ricinoleate                                                                         |         | 0.5  |
| Triethanolamine                                                                                     |         | 2    |
| Heterocopolymer of ethylene oxide-1,2-propylene oxide (72/25) having a viscosity of 450 at 100° F.  | 50      | 5    |
| Water                                                                                               | Balance |      |
| Composition E:                                                                                      |         | 55   |
| Dipotassium alpha-chloroethyl phosphonate                                                           | 4       |      |
| Diethanolamine stearate                                                                             |         | 0.1  |
| Diethanolamine                                                                                      |         | 2    |
| Heterocopolymer of ethylene oxide-1,2-propylene oxide (72/25) having a viscosity of 450 at 100° F.  | 60      | 10   |
| Water                                                                                               | Balance |      |
| Composition F:                                                                                      |         | 60   |
| Dilithium chloromethyl phosphonate                                                                  | 3       |      |
| Triethanolamine oleate                                                                              |         | 0.1  |
| Triethanolamine                                                                                     |         | 1.5  |
| Heterocopolymer of ethylene oxide-1,2-propylene oxide (72/25) having a viscosity of 1400 at 100° F. | 65      | 3.0  |
| Water                                                                                               | Balance |      |
| Composition G:                                                                                      |         | 70   |
| Sodium alpha-chloropropyl phosphonate                                                               | 4       |      |
| Triethanolamine ricinoleate                                                                         |         | 0.5  |
| Triethanolamine                                                                                     |         | 2    |
| Heterocopolymer of ethylene oxide-1,2-propylene oxide (72/25) having a viscosity of 450 at 100° F.  | 75      | 5    |
| Water                                                                                               | Balance |      |

The outstanding properties of compositions of this invention are demonstrated by results obtained for the following tests:

(1) Four-Ball Machine Tests are described in the Journal of the Institute of Petroleum Technology, pages 206-229, April 1946.

(2) Rust tests: (A) Freshly sand blasted iron strips were partially immersed in test fluids for 24 hours and amount of rust noted and rated:

A=no rust

B=slight rust in vapor space only

C=slight rust in liquid, moderate in vapor

D=moderate in both phases

E=heavy in both phases

(B) Test fluids were circulated over fresh steel turnings and time of rusting noted.

(3) Foam test: Test fluid stirred for 1 minute in Waring Blender and foam and liquid volume noted.

(4) Storage stability: Amount of phase separation noted of test fluids when stored over a temperature range of 5° C. to room temperature.

(5) Machining tests: Thread test—30 inches of 1/2-in.-13 pitch thread were cut with high speed steel, tangent chasers at 65 s.f.p.m., with different test fluids. Surface conditions of thread and size of weld (pick-up) on chaser flank were noted and rated where 0=excellent threads and no pick-up and 100=poor threads and heavy pick-up.

Lathe tool friction test—In heavy duty lathe turning of AISI-4340 alloy steel, the tool-chip coefficient of friction was equal to that of a premium quality petroleum cutting oil containing sulfur, chlorine and fatty additives.

Compositions A, B and D were diluted with 5 parts of water each, in rust test (A) and gave rating of A, and in rust test (B) were effective as rust inhibitors for over 13 days with no sign of rusting of the steel turnings. On the other hand a commercial oil-in-water emulsion, cutting fluid (X) containing sodium sulfonate and triethanolamine, gave a rust rating of D in test (A) and caused rusting in test (B) after 2 days. In the forming test, the above compositions A, B and D of the present invention were foam resistant whereas, composition X formed a heavy foam. Compositions A, B and D of the present invention were storage stable for over 28 days at room temperature and at 5° C., whereas with composition X, phase separation was noted after 3 days. In the threading test compositions A, B and D gave demerit ratings of 10 to 30, whereas, composition X gave ratings of 80-85. In the Four-Ball Test compositions A, B and D gave weld loads of 600 and 1000 kg. over a 5 second period, whereas, composition X gave weld loads of 200 kg.

Compositions of this invention can be applied with excellent results to heavy duty, high speed cutting operations where cooling and lubrication of the tool and work piece under adverse conditions are encountered. Metals machined with the aid of fluids of this invention have excellent surface finish and are free rust and stains.

We claim as our invention:

1. An aqueous metal working lubricant comprising a major amount of water and from about 0.5% to about 15% by weight of each of (1) water-soluble dialkali metal salt of chloro C<sub>1-4</sub> alkyl phosphonic acid, (2) an alkanolamine salt of a C<sub>12-20</sub> unsaturated fatty acid, (3) free alkanolamine and (4) a water-soluble heterocopolymer of a mixture of randomly distributed ethylene and propylene oxides having a molecular weight of from 250 to about 1500.

2. An aqueous metal working lubricant comprising a major amount of water and from about 2% to about 10% by weight each of (1) a water-soluble dialkali metal salt of chloromethyl phosphonic acid, (2) an ethanolamine salt of fatty acid selected from the group consisting of saturated or unsaturated fatty acids having from 12 to 18

carbon atoms, (3) ethanolamine, and (4) a water-soluble heterocopolymer of a mixture of randomly distributed ethylene and propylene oxides having a molecular weight of from 250 to about 1500.

3. An aqueous metal working lubricant comprising a major amount of water containing from about 2% to about 10% each of dipotassium chloromethyl phosphonate, triethanolamine oleate, triethanolamine and a water miscible heterocopolymer of ethylene oxide and propylene oxide in the mol ratio of from 75:25 to 10:90, respectively, having the molecular weight of from about 250 to about 1500.

4. An aqueous metal working lubricant comprising a major amount of water containing from about 10% each of disodium chloromethyl phosphonate, triethanolamine oleate, triethanolamine and a water miscible heterocopolymer of ethylene oxide and propylene oxide in the mol ratio of from 75:25 to 10:90, respectively, having a molecular weight of from about 250 to about 1500.

5. An aqueous metal working lubricant comprising a major amount of water containing from about 2% to about 10% each of dilithium chloromethyl phosphonate, triethanolamine oleate, triethanolamine and a water miscible heterocopolymer of ethylene oxide and propylene oxide in the mol ratio of from 75:25 to 10:90, respectively, having a molecular weight of from about 250 to about 1500.

6. A water base metal working lubricant comprising

about 3% to 8% dipotassium chloromethyl phosphonate, about 0.5% to 1% of triethanolamine oleate, from about 2 to 4% triethanolamine and from about 2% to 10% of heterocopolymer of ethylene oxide and propylene oxide in the mol ratio of from 75:25 to 10:90, respectively, having a molecular weight of from about 250 to about 1500.

#### References Cited by the Examiner

##### UNITED STATES PATENTS

|           |       |                   |       |             |
|-----------|-------|-------------------|-------|-------------|
| 2,311,306 | 2/43  | Ritchey           | ----- | 252—32.5    |
| 2,599,807 | 6/52  | Bersworth         | ----- | 260—500     |
| 2,625,509 | 1/53  | Laug              | ----- | 252—34.7    |
| 2,777,819 | 1/57  | Williams et al.   | ----- | 252—32.5    |
| 2,858,332 | 10/58 | Watson et al.     | ----- | 252—32.5 X  |
| 2,874,120 | 2/59  | Watson et al.     | ----- | 252—32.5    |
| 2,874,184 | 2/59  | Van Winkle et al. | ----- | 260—500     |
| 2,922,810 | 1/60  | Toy et al.        | ----- | 260—461.310 |
| 2,960,522 | 11/60 | Toy et al.        | ----- | 260—461.310 |
| 2,981,686 | 4/61  | Reamer            | ----- | 252—49.3 X  |

##### FOREIGN PATENTS

|         |      |                |
|---------|------|----------------|
| 539,293 | 9/41 | Great Britain. |
|---------|------|----------------|

25 DANIEL E. WYMAN, Primary Examiner.

JULIUS GREENWALD, Examiner.